

## UNITED STATES PATENT OFFICE

1,988,441

## MANUFACTURE OF VULCANIZED FIBER

John K. Anthony, Cleveland Heights, Ohio, assignor to Horace B. Fay, Cleveland, Ohio

No Drawing. Application March 24, 1931, Serial No. 525,040

3 Claims. (Cl. 154—50)

In the manufacture of vulcanized fiber, it has been customary to treat cellulose sheets with a hydrating agent, as zinc chloride or sulphuric acid, and then ply the sheets together to build up the thickness desired, and subsequently wash out the hydrating agent. This latter operation is tedious, since the hydrating agent on the interior of the mass must be removed by osmotic action in the washing bath, and this requires much time in the case of thicker stock even months of continued washing. All this not only adds to the extent of plant equipment in the washing department, but also ties up a large stock of material in transit through the process, thereby adding correspondingly to the overhead, as well as the general complication of the process. A procedure making possible the avoidance of such difficulty in the elimination of the treating agent, and making possible the formation of vulcanized fiber of any desired thickness, irrespective of limitations in elimination of the treating agent, is accordingly a fundamental desideratum and of particular importance.

To the accomplishment of the foregoing and related ends, the invention, then, comprises the features hereinafter fully described, and particularly pointed out in the claims, the following description setting forth in detail certain illustrative embodiments of the invention, these being indicative, however, of but a few of the various ways in which the principle of the invention may be employed.

In proceeding in accordance with the invention, cellulose, conveniently in sheet form, usually as felted out in paper-like condition, is subjected to the action of a hydrating agent, as zinc chloride, zinc iodide, sulphuric acid, etc. Most usually, a zinc chloride solution is desirable, this being of rather high concentration, this being about 70° Bé., or slightly more or less, in accordance with temperatures and particular character of product desired. The cellulose sheet, in one or more plies is fed through a bath of such hydrating agent, at a rate of travel to give a treating action of, for example, 3 to 10 minutes, depending upon the thickness of the sheet, and the concentration of the bath. From the hydrating bath, the sheet material is then conducted, surplus solution being eliminated by squeeze-rolls for instance, to a water-washing bath. Conveniently, this may be of a character such that the sheet material passes therethrough in zig-zag course, guided by suitable rollers, and preferably, the wash-water is directed counter-currently. A plurality of successive vats may be thus employed.

After washing for several hours, the exact time depending upon the thickness of the sheet, and the concentration of the original treating bath, the sheet material is sufficiently freed from residual hydrating agent. Surplus water is then eliminated. The sheet material may be, in fact, quite largely dried, although it is advisably not dried to such a complete extent as to cockle. Freed of surplus water, the sheet material is then plied together with interposed material causing adhesion. This may be provided, for instance, by passing the sheet-stock through a cupro-ammonium solution, made by dissolving copper hydrate in ammonia, or by dissolving metallic copper in the presence of air, in ammonia. More or less concentration of the ammonia is desirable, depending upon the extent to which residual water remains in the sheet-stock. By passing the stock through the cupro-ammonium bath and then plying together, the product may be built up to such thickness as desired in any particular case. Drying is advisably carried out under tension or pressure, to insure smoothness of product.

Among other convenient bonding agents, are such materials as proteinous agents, shellac in alcoholic solution, other resins, artificial resinoids such as phenol-aldehyde condensation products, and the like. The latter may be applied as thinned by a solvent or cutting agent, for instance ethyl alcohol or methanol being feasible with the commoner artificial resinoids. With any such bonding agents, the vulcanized-fiber sheet material as coming from the washing and surplus-water eliminating stage, is simply passed through a bath of such bonding material, and is plied together to the desired thickness, and dried, desirably under tension or pressure. Heat may be applied, particularly with the phenol-aldehyde resin binders. In some cases, a further final finishing pressing in a heated platen press or the like is advisable.

In such manner, the vulcanized fiber product may be formed to any desired thickness, and irrespective of the thickness, it is seen that the residual zinc chloride or other hydrating agent can be completely washed out, thereby affording a staple and durable product irrespective of its thickness. Moreover, since the washing is performed on unit-thickness material, the operation proceeds rapidly, and requires no more time for products ultimately made of greater thickness. Furthermore, it will be noticed that whereas heretofore vulcanized fiber has always been open to the objection of hydroscopicity, the material being inherently water-attracting, in accordance

with the present process where it is bonded by an extraneous bonding agent, water-proof materials may be so employed, as indicated in some of the above instances, and a water-resistant vulcanized fiber product may be had in one simple and direct operation.

Other modes of applying the principle of the invention may be employed, change being made as regards the details described, provided the features stated in any of the following claims, or the equivalent of such, be employed.

I therefore particularly point out and distinctly claim as my invention:

1. Vulcanized fiber bonded while containing disseminating water, by a water-borne agent which is water-insoluble as finally dehydrated.

2. Vulcanized fiber having initial hydrating agent eliminated and being bonded together by an extrinsic initially water-soluble water-proof agent applied while the fiber contains disseminating moisture.

3. Vulcanized fiber having initial hydrating agent eliminated, and while the fiber contains moisture being treated with a strong cuproammonium solution.

JOHN K. ANTHONY.